

Nov. 8, 1932.

M. I. FLETCHER

1,886,798

PRESTARCHED LINING FOR CUFFS AND OTHER APPAREL

Filed April 21, 1930



*Fig. 2.*



Inventor

*Maud I. Fletcher.*

*By*  
*Lacey, Lacey,*

Attorneys

## UNITED STATES PATENT OFFICE

MAUD I. FLETCHER, OF DOUGLAS, ARIZONA

## PRESTARCHED LINING FOR CUFFS AND OTHER APPAREL

Application filed April 21, 1930. Serial No. 446,120.

This invention relates to apparel and more particularly to a lining for use when forming cuffs, collars and other apparel for which it may be found suitable.

At the present time it is customary to provide cuffs and collars with an inner lining in order to impart a desired stiffness and body to the cuff or collar and after the shirt to which cuffs and collars are attached have been completed apply starch to the cuffs and collars before ironing them. This requires the services of employees to carry out the starching operation and also causes loss of time as the starch must dry before the cuffs and collars can be ironed. It also necessitates keeping starch on hand and providing storage space for the same which could be used for other purposes. It will thus be seen that the present method of starching cuffs and collars involves considerable loss in time and extra expense to a manufacturer.

Therefore, one object of the invention is to provide linings or material from which linings may be cut by a manufacturer, in which the fabric from which the linings are made has been previously starched but which is supplied to the manufacturer in a rough dried condition so that it will be sufficiently soft to permit it to be easily cut and passed through a sewing machine.

Another object of the invention is to provide a prestarched material from which linings may be cut thereby making it unnecessary to apply starch to a cuff or collar after forming the same and thereby eliminating likelihood of starch being applied and soiling parts of a garment adjoining the collar and cuffs or parts adjoining any parts which should be starched.

Another object of the invention is to provide a prestarched lining in which the starch contains paraffin or an equivalent lubricant in order to cause an iron to slide easily over a cuff or collar while ironing the same and to further so form the starch that ingredients of the formula used will cause the collars or cuffs to be whitened and the starch prevented from freezing if the fabric after being starched is dried in a freezing atmosphere.

The invention is illustrated in the accompanying drawing, wherein,

Figure 1 is a perspective view of a cuff having a lining formed of fabric prestarched in accordance with this invention, and

Figure 2 is a sectional view through the cuff taken on the line 2—2 of Figure 1.

While the prestarched fabric has been shown used as a lining for a cuff it is to be understood that it may be used as a lining for a collar or any other apparel which should be starched before it is placed on sale and in fact fabric from which the apparel itself is formed may be prestarched instead of merely the lining in case the entire apparel is to be delivered to a merchant in a starched and ironed condition.

Referring to the accompanying drawing, the numeral 1 indicates a cuff sewed to a shirt sleeve 2 in the usual manner and this cuff is provided with a lining 3 preferably formed of thicker fabric than that from which the body portion of the cuff is formed. The lining may consist of a single layer of fabric or a plurality of layers as shown at 4 in Figure 1. It will also be obvious that if the lining consists of more than one layer it may be formed from a strip or sheet of fabric folded upon itself to provide the desired number of layers or consist of separate sheets of fabric.

The fabric from which the linings are cut is to be supplied to a manufacturer in bulk or the linings may be previously cut and delivered to the manufacturer in the form of blanks ready for use. In either case the fabric from which the linings are formed is to be starched before it is delivered to the manufacturer. While a cold starch may be used it is preferred to use a cooked starch. This starch may be made in accordance with any formula but the following formula is preferably followed and it is to be understood that the ingredients will be proportionately increased if a larger quantity of starch is required.

When making the starch, wet and mix two tablespoons of starch and one teaspoon of salt in one-fourth pint of cold water. After the starch and salt have been thoroughly mixed in the cold water, add one pint of boiling

water in which has been dissolved one teaspoon of borax and then boil for one minute, remove from the fire and add one-half teaspoon of paraffin, oil or clear grease to serve as a lubricant.

5 Instead of the above, a flour starch may be used made in accordance with the following formula. Mix three tablespoons of flour and one-half teaspoon of salt in one-fourth pint of cold water and then add one pint of boiling water containing a teaspoon of borax.

10 After boiling the above for three minutes remove from the fire and add one-half teaspoon of paraffin, or an equivalent lubricant.

15 After the starch has been made it is applied to the lining fabric or blank in the usual manner and then the starched fabric is stretched and allowed to dry without being ironed. Therefore, the fabric or blank will be delivered to the manufacturer in a rough dry 20 state and will be sufficiently soft to permit linings to be cut from the fabric, and the cuffs or collars sewed in the usual manner without interference by a stiff lining.

25 After the cuff or collar has been completed it is dampened or steamed in order to moisten the starched lining and ironed in the usual manner. When the starch is dampened and the cuff or collar ironed the fabric from 30 which the body portion of the cuff or collar is formed adheres closely to the lining and forms a stiff collar or cuff without any danger of starched spots appearing. Of course, it is not necessary to apply starch to the cuff

35 or collar after it has been completed as the lining is impregnated with starch. The borax mixed with the boiling water when making the starch has a tendency to make white goods whiter and protect fast colors 40 and fine fabrics and the salt prevents the starch from freezing in case the starched fabric is dried in a freezing atmosphere. The paraffin serves as a lubricant to cause an iron to slide easily when ironing the cuff or 45 collar.

50 This starch washes out when the shirt or collar is laundered and therefore a cuff or collar formed as set forth above must be starched in the usual manner when laundered after being worn.

Having thus described the invention, I claim:

55 1. The method of forming cuffs and collars consisting of cutting a lining from a rough dried fabric impregnated with a starch soluble in water, forming a sheath of unstarched fabric, disposing the lining within the sheath and stitching marginal portions of the sheath and lining, moistening the finished article, and ironing the same.

60 2. A method of forming cuffs and collars consisting of forming a sheath of unstarched fabric, placing within the sheath a lining of 65 rough dried fabric impregnated with a starch

soluble in water, stitching marginal portions of the sheath and lining together, moistening the finished article, and ironing the same.

In testimony whereof I affix my signature.

MAUD I. FLETCHER. [L. S.]

70

75

80

85

90

95

100

105

110

115